

No. 627,855.

Patented June 27, 1899.

G. F. KEY.

PROCESS OF REFINING IRON.

(Application filed Mar. 10, 1898.)

(No Model.)

2 Sheets—Sheet 1.



Fig. 1.



Fig. 5.

Witnesses:

*John W. Smith*  
A. S. Shadley

Inventor:

George F. Key,  
By *Maguire & Son*  
Attorneys.

No. 627,855.

Patented June 27, 1899.

G. F. KEY.

PROCESS OF REFINING IRON.

(Application filed Mar. 10, 1898.)

(No Model.)

2 Sheets—Sheet 2.

Fig. 2.



Witnesses:

*John R. Smith*

A. Barthel

Inventor:

*George F. Key*

*By the Assignee*

Attorneys:

# UNITED STATES PATENT OFFICE.

GEORGE F. KEY, OF ANN ARBOR, MICHIGAN.

## PROCESS OF REFINING IRON.

SPECIFICATION forming part of Letters Patent No. 627,855, dated June 27, 1899.

Application filed March 10, 1898. Serial No. 673,311. (No specimens.)

*To all whom it may concern:*

Be it known that I, GEORGE F. KEY, a citizen of the United States, residing at Ann Arbor, in the county of Washtenaw and State 5 of Michigan, have invented certain new and useful Improvements in Processes of Refining Iron, of which the following is a specification, reference being had therein to the accompanying drawings.

10 This invention is especially designed for the purification of iron rich in phosphorus; and the object is to make iron manufactured from so-called "non-Bessemer" ores equally commercially available for the manufacture of 15 steel as iron made from Bessemer ores and which is convertible into steel by the Bessemer process.

To this end my improvement is based upon the general conclusions obtained in the practice of different processes that when phosphorus is present in a melted mixture of iron, iron oxid and ferrous silicate, or any suitable basic material, the tendency of the phosphorus is to become oxidized and converted into 25 phosphate, which separates in the slag, leaving a purer iron, while on the other hand if the cinder is mainly silicate or of an acid type the tendency is the other way—that is, part of the metallic iron becomes oxidized while 30 the phosphate is reduced, thus increasing the amount of phosphorus in the iron. Thus when plenty of ferric oxid is present and the mixture has a strong basic character phosphorus is largely removed from the molten 35 metal, while on the other hand in the ordinary Bessemer blowing process the first action of the oxygen of the blast acts on the silicon rather than on the iron, and in consequence a highly-silicious cinder results, so 40 that removal of phosphorus by oxidation becomes impracticable. The temperature also influences the reaction of the iron oxid on phosphorus, the higher the temperature the more pronounced apparently being the tendency of the metal to retain the phosphorus. 45 Based on these considerations I accomplish the purifications in the following manner:

50 Into the molten metal from the cupola or blast furnace is introduced in intimate mixture basic material in a finely-divided state. This mixture then is atomized in a highly-oxidizing atmosphere in presence of superheated

steam, and into the bath resulting from this treatment air is then blown for about the same period as in the converter treatment. 55 The success of this operation depends upon the complete atomizing. The ordinary spraying as practiced in some processes heretofore is not efficient, and it cannot be successfully atomized unless the molten metal is first 60 mixed with the finely-divided basic material, and it requires also a strong blast of steam, which if the basic material were introduced separately would blow it out of the furnace. While the atomized mixture is suspended, it 65 is in contact with the steam and with a highly-oxidizing atmosphere, which is maintained by injecting preheated air through a bunch of twyers.

The introduction of the basic material is 70 preferably accomplished by mixing powdered limestone directly into the stream of molten metal as it flows into the atomizing-chamber.

The effect of atomizing the molten metal in a highly-oxidizing atmosphere is that a considerable portion of the metal is oxidized, the presence of steam contributing to make ferric oxid, (which makes a more fusible slag,) and the bath resulting therefrom becomes thus intimately mixed with these oxid and 80 with the basic material introduced with the molten metal, and in the subsequent blowing instead of oxid being formed (as in the converter) the oxid already present react not only to a certain extent upon the silicon, but 85 mostly upon the phosphorus, and silicates and phosphates are formed separate with the slag, while the carbon burns out. In this manner the eliminations of phosphorus from molten metal not too highly phosphorized can 90 be satisfactorily and speedily accomplished in one operation, and the metal will be found surprisingly homogeneous.

If necessary, the operation can be repeated, (in the presence of heat to keep the metal 95 fluid,) or for the further treatment the open-hearth process may be more or less closely followed, according to the desired quality of steel, thereby shortening the time to one-fourth the time of what the process now requires. Besides the saving in time the result is superior, as the prolonged treatment by the open-hearth process alone results in loss of metal and the introduction of certain im-

purities from the lining and from the furnace-gases.

To carry out my process in the best manner, I have devised the following apparatus, as 5 shown in the drawings, in which—

Figure 1 is a vertical longitudinal section of the furnace. Fig. 2 is a front elevation thereof with the cupola and rotary screen removed, and Fig. 3 is an inner face view of the gas-10 chamber.

15 A is the reducing-chamber, having the usual basic lining and formed with a forwardly-inclined bottom and communicating at the rear end into a suitable stack B for the exit of the waste gases. In the front end is arranged the chamber C, which communicates through a suitable pipe D with a supply of air under pressure and preferably through a pipe D' with a supply of gas. The chamber C communicates by a series of openings or twyers E into the furnace-chamber, and above the same is arranged a blast-nozzle P, through which a current of steam of suitable volume and force may be introduced. In the top of the chamber, above this blast-pipe, is placed a hopper 25 G, terminating in an orifice H. The front end of the furnace has a trap-door J, in which is a tap-hole I. This door may be used for cleaning out the furnace. In the top is a suitable 30 feed-opening K, provided with a removable door D. Near the bottom, in one or both sides, are arranged a series of twyars M, suitably inclined to discharge into the bath of metal collected at the bottom of the furnace.

35 N is a rotary screen placed above the hopper G and serving to receive the powdered limestone or other basic material used by my process and which by agitating the screen is made to drop through a slot in the outer casing into the hopper G.

40 I also preferably provide means for introducing heat into the furnace, which may be accomplished by providing an aperture O in the face-plate, through which an oil-burner 45 may be introduced.

In carrying out my process with this apparatus I preferably locate the furnace in such relation to the cupola or blast furnace that

the molten metal may be run directly into the hopper G, from whence it flows in a thin 50 stream through the orifice H directly across the path of the steam from the nozzle F, the blast of which strikes the liquid metal and completely atomizes it and disperses it through the whole extent of the chamber in 55 the furnace, which to this end is largely extended in the direction in which the blast strikes. At the same time preheated air is injected through the twyars E, so that in the whole interior of the furnace a highly-oxidizing 60 atmosphere is maintained. Simultaneously with the introduction of the metal into the hopper G the screen is agitated, and the powdered basic material dropping into the vortex of the metal in the hopper is drawn in 65 with it and becomes intimately mixed with it and equally atomized with the metal. As soon as the metal has collected again the bath is then blown the usual time required to effect the reaction, after which the metal is 70 drawn off. During the treatment a rise in temperature takes place, and as the operation is quickly accomplished no extra heat is ordinarily required, except that at the start the furnace should be preheated, which can be 75 accomplished with the means described. By providing the chamber C with a separate connection for gas the furnace can be readily connected to one of the character of the open-hearth furnace, if desired, for a further treatment 80 of the metal.

What I claim as my invention is—

The herein-described process of refining pig-iron which consists in intimately mixing the molten metal with finely-divided limestone or other basic material, atomizing this mixture in a highly-oxidizing atmosphere of air and steam, collecting the atomized mixture into a bath and then blowing the same with air, or other refining purifying-gas. 85

In testimony whereof I affix my signature in presence of two witnesses.

GEORGE F. KEY.

Witnesses:

M. B. O'DOGHERTY,  
OTTO F. BARTHEL.